# EUROPEAN PATENT SPECIFICATION

(11) **EP 3 625 808 B1**
(45) Date of publication and mention of the grant of the patent: **13.04.2022**
(21) Application number: 18731577.5
(22) Date of filing: 17.05.2018
(51) Int. Cl.: H01F 1/147, H01F 1/153, C22C 38/00, C22C 38/02, C22C 38/04, C22C 38/06, C22C 38/08, C22C 38/10, C22C 38/12, C22C 38/14, C22C 38/18, C22C 38/30, C22C 38/32, C22C 38/34, C21D 8/12

(54) **FE-SI BASE ALLOY AND METHOD OF MAKING SAME**
LEGIERUNG AUF FE-SI-BASIS UND HERSTELLUNGSVERFAHREN DAFÜR
ALLIAGE À BASE DE FE-SI ET SON PROCÉDÉ DE FABRICATION

(30) Priority: 17.05.2017 US 201762507415 P
(43) Date of publication of application: 25.03.2020
(73) Proprietor: CRS Holdings, LLC, Wilmington, DE 19801 (US)
(72) Inventor: CHINNASAMY, Chins, Lancaster, PA 17601 (US); KERNION, Samuel J., Lancaster, PA 17601 (US); FITTERLING, Eric, Macungie, PA 18062 (US); POLAR-ROSAS, Alberto, Reading, PA 19606 (US); WANG, Tao, Reading, PA 19608 (US)
(74) Representative: Mewburn Ellis LLP
(86) International application number: PCT/US2018/033155
(87) International publication number: WO 2018/213556

(56) References cited:
- EP-A1- 1 108 794
- EP-A1- 2 025 766
- EP-A1- 2 055 797
- EP-A1- 2 933 348
- US-A- 4 337 087
- US-A1- 2012 262 266

## Description

### BACKGROUND OF THE INVENTION:

### Field of the Invention:

This invention relates to soft magnetic alloys containing Fe and Si and in particular, to a soft magnetic Fe-Si alloy containing one or more additive elements to benefit the ductility and formability of the alloy.

### Description of the Related Art:

Iron-silicon (Fe-Si) steel sheet containing 6.5-7% silicon features excellent magnetic properties, including greatly reduced core loss at high frequencies and very low magnetostriction compared to Fe-Si steel sheet containing less than 4% Si. Because of those characteristics, Fe-Si steel sheet containing nominal 6.5% Si has high potential for use in various electrical devices and shielding applications, including cores for transformers and the stators and rotors of motors and generators. Such a material would offer advantages of weight reduction, vibration reduction, and noise reduction, as well as electric power savings. However, the presence of ordered phases in the nominal 6.5% Si steel alloy, namely the B2 (FeSi) and D0₃ (Fe₃Si) phases, causes embrittlement of the steel alloy at room temperature. The lack of adequate ductility and formability makes it difficult to process the alloy into thin sheet, strip, or foil form by conventional processes such as cold rolling, warm rolling, and hot rolling. When the Si content is more than 4 wt. %, the percent elongation decreases rapidly and conventional cold rolling techniques cannot be readily used.

In order to avoid the adverse effect of higher silicon on the formability of the steel alloy, special processing techniques have been used. Such techniques include strict temperature controls and strict limitations on reductions in thickness during hot, warm, and/or cold working steps. Another technique includes the application of a siliconized layer to Fe-Si steel strip by chemical vapor deposition (CVD). However, such techniques unduly increase the cost of producing Fe-Si steel strip and sheet.

In view of the state of the art, it would be desirable to be able to produce Si-rich, Fe-Si electrical steel strips and sheets of various thicknesses that have excellent magnetic characteristics such as high saturation induction, low coercivity, high permeability, high electrical resistivity, low magnetostriction, and low core loss at high frequencies. It would also be desirable to produce such Si-rich, Fe-Si alloy products by using conventional metallurgical techniques and processes to obtain the above-described magnetic characteristics for use in the production of soft magnetic laminated cores with reduced weight, low energy losses, and low cost for the next generation of electromagnetic devices such as motors, generators, transformers, inductors, choke coils, actuators, fuel injectors, compressors, and other electromotive devices.

### SUMMARY OF THE INVENTION:

In accordance with a first aspect of the present invention there is provided an alloy according to claim 1 that resolves the processing disadvantages of the known Fe-Si materials. The alloy is further defined by the following weight percent ranges for the constituent elements.

| | Broad | Intermediate | Preferred |
|---|---|---|---|
| Si | 4-7 | 4-7 | 4-7 |
| M | 0.1-7 | 0.5-6 | 1-5 |
| L | 0.1-7 | 0.5-7 | 0.75-6 |
| M' | up to 7 | up to 5 | 0.1-3 |
| M" | up to 7 | 5 max. | 3 max. |
| R | up to 1 | up to 1 | up to 1 |

| | | | |
|---|---|---|---|
| The balance of the alloy is iron and usual impurities. The alloy has a microstructure that contains 75-100% by volume of disordered bcc phase. | | | |

In accordance with a second aspect of the present invention there is provided a thin-gauge article according to claim 8.

In accordance with another aspect of the present invention there is provided a method of making a steel alloy product from a soft magnetic alloy according to claim 9.

The foregoing tabulation is provided as a convenient summary and is not intended to restrict the ranges of the elements for use solely within the broad, intermediate, and preferred embodiments as set forth in the table. Thus, one or more of the ranges of the broad, intermediate, or preferred embodiments can be used with one or more of the ranges of a different embodiment for the remaining elements. In addition, a minimum or maximum for an element of one of the broad, intermediate, or preferred compositions can be used with the minimum or maximum for the same element in a different embodiment.

Here and throughout this specification the following definitions apply. The term "percent" and the symbol "%" mean weight percent or mass percent unless otherwise indicated. The term "vol.%" means percent by volume. The term "thin gauge" or "thin-gauge" means a thickness of not more than about 0.08 inches (2.03 mm). The term "additive element" means one or more elements added to the base alloy in an amount sufficient to provide a desired effect on one or more properties.

### DETAILED DESCRIPTION:

The alloy according to this invention is an iron-silicon base alloy that can be defined by having the following general chemical formula:

Fe_{100-a-b-c-d-e-f}SiₐM_{b}L_{c}M'_{d}M"ₑR_{f}.

Silicon: This alloy contains at least about 4% silicon to benefit the magnetic properties provided by the alloy. In particular, silicon reduces the core loss at high operating frequencies and significantly lowers the magnetostriction of the alloy. Too much silicon promotes the formation of the ordered phases B2 and D0₃, both of which result in embrittlement of the alloy and a consequent loss of ductility. Therefore, the alloy contains not more than about 7% silicon to inhibit the formation of such phases.

M: M is one or both of chromium and molybdenum. Chromium and molybdenum benefit the ductility of the alloy particularly at elevated temperatures at which elongated forms of the alloy are warm rolled. M retards the order-disorder transformation reaction during the cooling process. In this manner, the formation of ordered bcc phases such as B2 and D0₃ is inhibited. M also reduces the ductile-to-brittle transition temperature of the alloy which allows the alloy to be cold rolled at lower temperatures than the known Si-Fe alloys. Toward those ends, the alloy contains at least about 0.1% of one or both of chromium and molybdenum. Preferably, the alloy contains at least about 0.5% and for best results, at least about 1% Cr+Mo. Chromium and molybdenum are restricted to not more than about 6% in order to avoid an adverse effect on the magnetic properties provided by the alloy. Preferably, the alloy contains not more than about

L: L is cobalt, nickel, or a combination thereof. Cobalt and/or nickel are present in this alloy to benefit the soft magnetic properties provided by this alloy. More specifically, the L elements increase the Curie temperature of the alloy which extends its magnetic behavior over a broader temperature range. Cobalt and nickel also increase the magnetic saturation induction of the alloy, and provide an increase in permeability. Accordingly, the alloy contains at least about 0.1% and preferably at least about 0.5% of one or both of cobalt and nickel. Good results have been obtained when this alloy contains at least about 0.75%, for example, at least about 0.85% Co+Ni. For best results, the alloy contains at least about 1% Co+Ni. Too much cobalt and/or nickel eventually increases the magnetocrystalline anisotropy and the magnetostriction of the alloy. Too much cobalt and/or nickel may also increase the core loss to an undesirable level. Therefore, the alloy contains not more than about 7%, and preferably contains not more than about 5% or 6% of Ni+Co.

M': M' is selected from the group consisting of aluminum, manganese, copper, germanium, gallium, and a combination thereof. Up to about 5% of M' may be present in this alloy to benefit the electrical and magnetic properties provided by the alloy. When present M' increases the electrical resistivity of the alloy, increases the magnetic permeability of the alloy, and lowers the coercive force. Preferably the alloy contains at least about 0.1% of M'. Too much M' adversely affects the magnetic properties of the alloy such as the magnetic saturation induction. Therefore, the alloy preferably contains not more than about 4% of M'.

M": M" is selected from the group consisting of titanium, vanadium, hafnium, niobium, tungsten, and a combination thereof. Up to about 7% of M" may be present in the alloy. When present M" benefits the ductility of the alloy by retarding the formation of embrittling ordered phases in the alloy when the alloy is cooled. Too much M" adversely affects the magnetic properties provided by the alloy, particularly the magnetic saturation induction provided by the alloy. Therefore, the alloy preferably contains less than about 5% and better yet less than about 3% of M".

R: R is one or more of the elements boron, zirconium, magnesium, phosphorus, and cerium. A small amount up to about 1% of R may present in this alloy for grain refinement and to strengthen grain boundaries in the alloy during the forming process, where a preferred grain size of ASTM 5 or finer is desired.

The balance of the alloy is iron and the usual impurities present in commercial Fe-Si alloys intended for similar use or service. Carbon, nitrogen, and sulfur are considered impurities in this alloy because they are known to form carbides, nitrides, carbonitrides, or sulfides. Such phases can adversely affect the magnetic properties that are characteristic of the alloy. Therefore, the alloy contains not more than about 0.1% carbon, not more than about 0.1% nitrogen, and not more than about 0.1% sulfur. Preferably, the alloy contains not more than about 0.005% each of carbon, nitrogen, and sulfur when the alloy includes carbide-, nitride-, carbonitride-, and/or sulfide-forming elements.

Because of the alloying of the additive elements L and M and the optional elements M', M", and R with Fe and Si, an alloy product according to the present invention contains at least about 75 vol.% of the disordered bcc phase. In a particular embodiment, the alloy product consists essentially of the disordered phase only, i.e., about 100 vol.% disordered bcc phase. It has been found that the presence of the disordered phase and a minimal amount of the ordered phase(s) might have beneficial effects on the plasticity of the alloy which results in improved formability, particularly cold formability. For most applications, the alloy product can be characterized by a microstructure containing disordered phases such as A2 in the range of 75 to about 100 vol.% whereby the magnetic properties of the alloy product are expected to be significantly improved relative to the known Fe-Si steel.

An intermediate form of alloy article according to this invention is produced in the form of thin-gauge sheets and strips having thicknesses of 0.0001 in. (2.54µm) to about 0.1 in. (2.54mm). Preferred thicknesses include 0.002 in. (0.0508 mm), 0.005 in. (0.127 mm), 0.007 in. (0.178 mm), 0.010 in. (0.254 mm), 0.014 in. (0.356 mm), 0.019 in. (0.483 mm) and 0.025 in. (0.635 mm). The width of the sheet or strip product depends on the application in which the alloy will be used. Typically, the alloy article would be about 0.5 to 40 inches (12.7 mm to 101.6 cm) in width for most applications.

The alloy article according to the present invention is preferably produced by first melting and casting the alloy into an ingot. After solidification, the ingot is thermomechanically processed as by hot and/or warm rolling to form an intermediate elongated product form having a thickness that is less than 2 in. (5.08 cm) but more than 0.05 in (1.27 mm). The hot or warm rolling step is carried out on the intermediate elongated product at in a temperature range that is selected to avoid tearing or cracking of the alloy. Preferably, hot rolling is carried out from a starting temperature of at least about 2102°F (1150°C) to a finish temperature not lower than about 1472°F (800°C). Warm rolling is preferably carried out from a starting temperature of at least about 1112°F (600°C) to a finish temperature of not less than about 302°F (150°C).

The intermediate elongated product is then cooled at a rate that is selected to inhibit the possible formation of ordered phases as the alloy cools to room temperature. The alloy is quenched in water, oil, gas, or in any other suitable quenching media from a temperature above the order-disorder transition temperature to avoid the formation of the ordered phases.

After the cooling step, the intermediate elongated form is further reduced in thickness by cold or warm rolling. The cold or warm rolling step is carried out in one or more passes to provide a second elongated form having the desired final thickness. The warm rolling step is conducted at temperatures similar to those described above for the thermomechanical working step. The second elongated form of the alloy can be further processed into useful finished or semi-finished parts such as laminations and other stampings. The finished or semi-finished parts can be heat treated to relieve stresses induced in the material during part fabrication or to promote phase transformation. The preferred heat treating temperature for stress relieving is in the range of 752-1382°F (400-750°C) and annealing time will depend on the product size and thickness. The alloy article can be annealed in an atmosphere such as hydrogen, vacuum, nitrogen, or a combination thereof. If desired, the second elongated form can be annealed either at a temperature above the order-disorder temperature or at a temperature below the order-disorder temperature depending on the product application in which the alloy strip product is intended for use. In any case the product should be cooled at a cooling rate high enough to maintain the desired microstructure and prevent further precipitation during cooling. The cooling rate is selected in agreement with the product size and thickness. The final product form is characterized by a good combination of mechanical and magnetic properties and high electrical resistivity.

The alloy of this invention and articles made therefrom can be produced by powder metallurgy techniques including powder spray and coating techniques known to those skilled in the art. It is also contemplated that parts and components can be made from the alloy powder by additive manufacturing processes.

Strip and sheet forms of the alloy of this invention can be further processed into useful finished or semi-finished parts such as laminations, stampings, and other forms for making electromagnetic devices including, but not limited to, electric motors and generators, transformers, inductors, choke coils, actuators, fuel injectors, and other electromotive devices. The preferred heat-treating temperature for stress relieving of finished or semi-finished parts is in the range of 752-1382°F (400-750°C) in an inert atmosphere. The stress relief annealing time will depend on the part size and thickness.

### WORKING EXAMPLES

In order to demonstrate the novel combination of properties provided by the alloy of this invention, 13 example heats were vacuum induction melted and cast as 40-lb. (18.1 kg) ingots. The weight percent chemistries of the heats are presented in Table 1 below. The balance of each composition is iron and usual impurities.

**Table 1**

| **Heat ID** | **Cr** | **Si** | **Co** | **Mn** | **B** | **Zr** | **Ni** |
|---|---|---|---|---|---|---|---|
| **Invention** | | | | | | | |
| 3036 | 3.25 | 5.15 | 1 | 0 | 0 | 0 | 0 |
| 3041 | 3.25 | 5.15 | 2.5 | 0.5 | 0 | 0 | 0 |
| 3042 | 3.25 | 5.15 | 4 | 1 | 0 | 0 | 0 |
| 3043 | 2.25 | 5.15 | 1 | 0.5 | 0 | 0 | 0 |
| 3044 | 2.25 | 5.15 | 2.5 | 1 | 0 | 0 | 0 |
| 3045 | 2.25 | 5.15 | 4 | 0.5 | 0 | 0 | 0 |
| 3046 | 1.5 | 5.15 | 1 | 1 | 0 | 0 | 0 |
| 3037 | 1.5 | 5.15 | 1.5 | 0 | 0 | 0 | 0 |
| 3047 | 1.5 | 5.15 | 4 | 0.5 | 0 | 0 | 0 |

| **Comparative** | | | | | | | |
|---|---|---|---|---|---|---|---|
| 3038 | 3.25 | 5.15 | 0 | 0 | 0.3 | 0 | 0 |
| 3039 | 3.25 | 5.15 | 0 | 0 | 0.5 | 0 | 0 |
| 3040 | 3.25 | 5.15 | 0 | 0 | 0.1 | 0 | 0 |
| 3058 | 2.26 | 5.15 | 0 | 0.16 | 0.02 | 0 | 0.01 |

| | | | | | | | |
|---|---|---|---|---|---|---|---|
| Heat Nos. 3036, 3041-3047, and 3037 are representative of the alloy according to the present invention. Heat Nos. 3038-3040 and 3058 are comparative alloys. | | | | | | | |

The ingots were processed to strip form as follows. The ingots were homogenized in the temperature range of 1652-2282°F (900-1250°C) for different durations that were selected based on the ingot size. The homogenized ingots were forged from 3.5-inch (8.9 cm) square to 5-inch (12.7 cm) width by 0.25-inch (0.635 cm) thickness slabs. The slabs were hot rolled in the range of 1472-2102°F (800-1150°C) to different thicknesses of strip. The hot rolled strips were reheated at a temperature of 392-1472°F (200-800°C) and warm rolled. After warm rolling to final thickness, the strips were cooled to room temperature. The final thickness (Thk.) of the strip sample from each heat is shown in Table 2 below in inches.

Also, set forth in Table 2 are the results of magnetic testing of the strip samples from the heats in Table 1 including the electrical resistivity in micro-ohm-centimeters (µΩcm)), maximum saturation induction (Bₘ) in kilogauss (wherein 1kG = 0.1T) coercivity in oersteds (wherein 1Oe = 79.6A/m), and DC permeability (unitless). Specimens in Condition A were warm rolled and not annealed. Specimens in Condition B were annealed at 1472°F (800°C) for 10 minutes after warm rolling.

**Table 2**

| | | **Elec. Res.** | | **DC Magnetic Properties** | | | | | |
|---|---|---|---|---|---|---|---|---|---|
| | **Thk. ↓** | | | **Induction (Bₘ)** | | **Coercivity (Hₘ)** | | **Permeability (µₘ)** | |
| **Heat ID** | **Cond. →** | **A** | **B** | **A** | **B** | **A** | **B** | **A** | **B** |
| | **Invention** | | | | | | | | |
| 3036 | 0.026 | 91 | 86 | 18.9 | 18.9 | 3.37 | 0.499 | 658 | 5125 |
| 3041 | 0.025 | 89.5 | 83 | 14.6 | 14.6 | 4.52 | 0.443 | 298 | 2743 |
| 3042 | 0.028 | 88 | 90 | 18.5 | 19.5 | 3.87 | 0.319 | 633 | 7247 |
| 3043 | 0.019 | 81.6 | 87 | 16.8 | 16.9 | 5.11 | 0.288 | 599 | 8058 |
| 3044 | 0.026 | 88 | 88 | 17 | 17.1 | 3.01 | 0.285 | 782 | 7910 |
| 3045 | 0.028 | 74.8 | 72 | 19.5 | 19.5 | 2.58 | 0.296 | 1006 | 11,100 |
| 3046 | 0.03 | 71.5 | 74.4 | 18.6 | 18.9 | 4.34 | 0.355 | 627 | 8756 |
| 3037 | 0.025 | 77.2 | 85 | 17.4 | 17.4 | 2.67 | 0.324 | 729 | 7219 |
| 3047 | 0.024 | 69 | 68 | 19.2 | 19 | 4.17 | 0.333 | 657 | 10,700 |

| | **Comparative** | | | | | | | | |
|---|---|---|---|---|---|---|---|---|---|
| 3038 | 0.014 | 99.5 | 99 | 16.6 | 15.2 | 3.57 | 0.667 | 869 | 4111 |
| 3039 | 0.026 | 94.8 | 96 | 19.2 | 18.7 | 3.82 | 0.5 | 828 | 6797 |
| 3040 | 0.027 | 103 | 102 | 12.3 | 12.4 | 4.78 | 0.77 | 416 | 3099 |
| 3058 | 0.03 | 82 | 91 | 17.8 | 18.3 | 3.27 | 0.525 | 698 | 4970 |

The terms and expressions which are employed in this specification are used as terms of description and not of limitation. There is no intention in the use of such terms and expressions of excluding any equivalents of the features shown and described or portions thereof. It is recognized that various modifications are possible within the invention described and claimed herein.

## Claims

1. A soft magnetic alloy having good formability, said alloy having the chemical formula
Fe_{100-a-b-c-d-e-f}SiₐM_{b}L_{c}M'_{d}M"ₑR_{f}
wherein M is one or both of Cr and Mo;
L is one or both of Co and Ni;
M' is selected from the group consisting of Al, Mn, Cu, Ge, Ga, and a combination thereof;
M" is selected from the group consisting of Ti, V, Hf, Nb, W, and a combination thereof;
R is selected from the group consisting of B, Zr, Mg, P, Ce, and a combination thereof; and
wherein Si, M, L, M', M", and R have the following ranges in weight percent:
| | |
|---|---|
| Si | 4-7 |
| M | 1-6 |
| L | 0.1-7 |
| M' | up to 5 |
| M" | up to 7 |
| R | up to 1 |
and the balance of the alloy is iron and usual impurities; and
wherein said alloy has a microstructure that contains 75-100% by volume of disordered bcc phase.

2. The soft magnetic alloy claimed in Claim 1 which contains at least 0.5% wt L.

3. The soft magnetic alloy claimed in Claim 1 which contains at least 0.75% 2. wt L and preferably not more than 6% wt L.

4. The soft magnetic alloy as claimed in Claim 2 which contains not more than 5%wt M".

5. The soft magnetic alloy claimed in Claim 4 which contains at least 0.75% wt L and preferably not more than 5% wt L.

6. The soft magnetic alloy claimed in Claim 1 wherein in weight percent:
| | |
|---|---|
| L | 0.75-5 |
| M' | 0.1-3 |
| M" | 3 max |

7. The soft magnetic alloy as claimed in any one of the preceding claims wherein the alloy contains not more than about 0.1% carbon, not more than about 0.1% nitrogen, and not more than about 0.1% sulfur when the alloy contains one or more elements that form or are likely to form carbides, nitrides, carbonitrides, and/or sulfides in the alloy.

8. A thin-gauge article formed from the alloy of claim 1, said thin-gauge article having a high magnetic saturation induction, high magnetic permeability, and good ductility.

9. A method of making a steel alloy product from a soft magnetic alloy comprising the steps of:
melting an alloy having the chemical formula
Fe_{100-a-b-c-d-e-f}SiₐM_{b}L_{c}M'_{d}M"ₑR_{f}
wherein M is one or both of Cr and Mo;
L is one or both of Co and Ni;
M' is selected from the group consisting of Al, Mn, Cu, Ge, Ga, and a combination thereof;
M" is selected from the group consisting of Ti, V, Hf, Nb, W, and a combination thereof;
R is selected from the group consisting of B, Zr, Mg, P, Ce, and a combination thereof; and
wherein Si, M, L, M', M", and R have the following ranges in weight percent:
| | |
|---|---|
| Si | 4-7 |
| M | 1-6 |
| L | 0.1-7 |
| M' | up to 5 |
| M" | up to 7 |
| R | up to 1 |
and the balance of the alloy is iron and usual impurities;
casting the alloy into an ingot;
thermomechanically processing said ingot to provide an intermediate elongated product form having a thickness less than about 2 in. (5.08cm);
cooling the intermediate elongated product; and then
mechanically working the intermediate elongated product form to produce a thin-gauge elongated product;
wherein the step of cooling the intermediate elongated product comprises cooling from a temperature above the order-disorder transition temperature by quenching to inhibit the formation of an ordered phase in the alloy.

10. The method claimed in Claim 9 wherein the step of thermomechanically working consists of hot rolling, warm rolling, or a combination of hot and warm rolling.

11. The method as claimed in Claim 9 wherein the mechanical working step consists of warm rolling, cold rolling, or a combination of warm and cold rolling the intermediate elongated product form.

## Patentansprüche

1. Weichmagnetische Legierung mit guter Formbarkeit, wobei die Legierung die chemische Formel
Fe_{100-a-b-c-d-e-f}SiₐM_{b}L_{c}M'_{d}M"ₑR_{f}
aufweist, worin
M eines oder beide aus Cr und Mo ist;
L eines oder beide aus Co und Ni ist;
M' aus der aus Al, Mn, Cu, Ge, Ga und einer Kombination daraus bestehenden Gruppe ausgewählt ist;
M" aus der aus Ti, V, Hf, Nb, W und einer Kombination daraus bestehenden Gruppe ausgewählt ist;
R aus der aus B, Zr, Mg, P, Ce und einer Kombination daraus bestehenden Gruppe ausgewählt ist; und
wobei Si, M, L, M', M" und R die folgenden Bereiche in Gewichtsprozent aufweisen:
| | |
|---|---|
| Si | 4-7 |
| M | 1-6 |
| L | 0,1-7 |
| M' | bis zu 5 |
| M" | bis zu 7 |
| R | bis zu 1 |
und der Rest der Legierung Eisen und übliche Verunreinigungen ist; und
wobei die Legierung eine Mikrostruktur aufweist, die 75-100 Vol.-% ungeordnete Bcc-Phase enthält.

2. Weichmagnetische Legierung nach Anspruch 1, die zumindest 0,5 Gew.-% L enthält.

3. Weichmagnetische Legierung nach Anspruch 1, die zumindest 0,75 Gew.-% L und vorzugsweise nicht mehr als 6 Gew.-% L enthält.

4. Weichmagnetische Legierung nach Anspruch 2, die nicht mehr als 5 Gew.-% M" enthält.

5. Weichmagnetische Legierung nach Anspruch 4, die zumindest 0,75 Gew.-% L und vorzugsweise nicht mehr als 5 Gew.-% L enthält.

6. Weichmagnetische Legierung nach Anspruch 1, wobei Folgendes die folgenden Bereiche in Gewichtsprozente aufweist:
| | |
|---|---|
| L | 0,75-5 |
| M' | 0,1-3 |
| M" | max. 3. |

7. Weichmagnetische Legierung nach einem der vorangegangenen Ansprüche, wobei die Legierung nicht mehr als etwa 0,1 % Kohlenstoff, nicht mehr als etwa 0,1 % Stickstoff und nicht mehr als etwa 0,1 % Schwefel enthält, wenn die Legierung ein oder mehrere Elemente enthält, die Carbide, Nitride, Carbonitride und/oder Sulfide in der Legierung bilden oder dazu neigen, diese zu bilden.

8. Dünnwandiges Erzeugnis, das aus einer Legierung nach Anspruch 1 gebildet wird, wobei das dünnwandige Erzeugnis eine hohe magnetische Sättigungsinduktion, eine hohe magnetische Permeabilität und eine gute Formbarkeit aufweist.

9. Verfahren zur Herstellung eines Stahllegierungsprodukts aus einer weichmagnetischen Legierung, das die folgenden Schritte umfasst:
das Schmelzen einer Legierung, die die folgende chemische Formel aufweist
Fe_{100-a-b-c-d-e-f}SiₐM_{b}L_{c}M'_{d}M"ₑR_{f}
worin
M eines oder beide aus Cr und Mo ist;
L eines oder beide aus Co und Ni ist;
M' aus der aus Al, Mn, Cu, Ge, Ga und einer Kombination daraus bestehenden Gruppe ausgewählt ist;
M" aus der aus Ti, V, Hf, Nb, W und einer Kombination daraus bestehenden Gruppe ausgewählt ist;
R aus der aus B, Zr, Mg, P, Ce und einer Kombination daraus bestehenden Gruppe ausgewählt ist; und
wobei Si, M, L, M', M" und R die folgenden Bereiche in Gewichtsprozent aufweisen:
| | |
|---|---|
| Si | 4-7 |
| M | 1-6 |
| L | 0,1-7 |
| M' | bis zu 5 |
| M" | bis zu 7 |
| R | bis zu 1 |
und der Rest der Legierung Eisen und übliche Verunreinigungen ist;
das Gießen der Legierung in einen Legierungsblock;
das thermomechanische Verarbeiten des Legierungsblocks, um eine längliche Zwischenproduktform mit einer Dicke von weniger als etwa 2 Zoll (5,08 cm) bereitzustellen;
das Abkühlen des länglichen Zwischenprodukts; und dann
das mechanische Bearbeiten der länglichen Zwischenproduktform, um ein längliches dünnwandiges Produkt herzustellen;
wobei der Schritt des Abkühlens des länglichen Zwischenprodukts das Abkühlen von einer Temperatur über der Ordnung-Unordnung-Übergangstemperatur durch Quenchen umfasst, um die Bildung einer geordneten Phase in der Legierung zu verhindern.

10. Verfahren nach Anspruch 9, wobei der Schritt des thermomechanischen Bearbeitens aus Heißwalzen, Warmwalzen oder einer Kombination aus Heiß- und Warmwalzen besteht.

11. Verfahren nach Anspruch 9, wobei der mechanische Bearbeitungsschritt aus Warmwalzen, Kaltwalzen oder einer Kombination aus Warm- und Kaltwalzen der länglichen Zwischenproduktform besteht.

## Revendications

1. Alliage magnétique doux ayant une bonne formabilité, ledit alliage ayant la formule chimique
Fe_{100-a-b-c-d-e-f}SiₐM_{b}L_{c}M'_{d}M"ₑR_{f}
dans lequel M est l'un de Cr et Mo, ou les deux ;
L est l'un de Co et Ni, ou les deux ;
M' est choisi dans le groupe constitué de Al, Mn, Cu, Ge, Ga, et d'une combinaison de ceux-ci ;
M" est choisi dans le groupe constitué de Ti, V, Hf, Nb, W, et d'une combinaison de ceux-ci ;
R est choisi dans le groupe constitué de B, Zr, Mg, P, Ce, et d'une combinaison de ceux-ci ; et
dans lequel Si, M, L, M', M", et R ont les plages suivantes en pourcentage en poids :
| | |
|---|---|
| Si | 4 à 7 |
| M | 1 à 6 |
| L | 0,1 à 7 |
| M' | jusqu'à 5 |
| M" | jusqu'à 7 |
| R | jusqu'à 1 |
et le reste de l'alliage est du fer et des impuretés habituelles ; et
ledit alliage ayant une microstructure qui contient 75 à 100 % en volume de phase bcc désordonnée.

2. Alliage magnétique doux selon la revendication 1, qui contient au moins 0,5 % en poids de L.

3. Alliage magnétique doux selon la revendication 1, qui contient au moins 0,75 % en poids de L et de préférence pas plus de 6 % en poids de L.

4. Alliage magnétique doux selon la revendication 2, qui ne contient pas plus de 5 % en poids de M".

5. Alliage magnétique doux selon la revendication 4, qui contient au moins 0,75 % en poids de L et de préférence pas plus de 5 % en poids de L.

6. Alliage magnétique doux selon la revendication 1, dans lequel, en pourcent en poids :
| | |
|---|---|
| L | 0,75 à 5 |
| M' | 0,1 à 3 |
| M" | 3 max. |

7. Alliage magnétique doux selon l'une quelconque des revendications précédentes, dans lequel l'alliage ne contient pas plus d'environ 0,1 % de carbone, pas plus d'environ 0,1 % d'azote, et pas plus d'environ 0,1 % de soufre lorsque l'alliage contient un ou plusieurs éléments qui forment ou sont susceptibles de former des carbures, des nitrures, des carbonitrures, et/ou des sulfures dans l'alliage.

8. Article de faible épaisseur formé à partir de l'alliage selon la revendication 1, ledit article de faible épaisseur ayant une induction de saturation magnétique élevée, une perméabilité magnétique élevée et une bonne ductilité.

9. Procédé de fabrication d'un produit en alliage d'acier à partir d'un alliage magnétique doux, comprenant les étapes consistant à :
faire fondre un alliage ayant la formule chimique
Fe_{100-a-b-c-d-e-f}SiₐM_{b}L_{c}M'_{d}M"ₑR_{f}
dans lequel M est l'un de Cr et Mo, ou les deux ;
L est l'un de Co et Ni, ou les deux ;
M' est choisi dans le groupe constitué de Al, Mn, Cu, Ge, Ga, et d'une combinaison de ceux-ci ;
M" est choisi dans le groupe constitué de Ti, V, Hf, Nb, W, et d'une combinaison de ceux-ci ;
R est choisi dans le groupe constitué de B, Zr, Mg, P, Ce, et d'une combinaison de ceux-ci ; et
dans lequel Si, M, L, M', M", et R ont les plages suivantes en pourcentage en poids :
| | |
|---|---|
| Si | 4 à 7 |
| M | 1 à 6 |
| L | 0,1 à 7 |
| M' | jusqu'à 5 |
| M" | jusqu'à 7 |
| R | jusqu'à 1 |
et le reste de l'alliage est du fer et des impuretés habituelles ; et
couler l'alliage en un lingot ;
traiter thermomécaniquement ledit lingot pour obtenir une forme de produit allongée intermédiaire ayant une épaisseur inférieure à environ 2 pouces (5,08 cm) ;
refroidir le produit allongé intermédiaire, puis usiner mécaniquement la forme de produit allongé intermédiaire pour produire un produit allongé de faible épaisseur ;
dans lequel l'étape de refroidissement du produit allongé intermédiaire comprend un refroidissement à partir d'une température supérieure à la température de transition ordre-désordre par trempe pour inhiber la formation d'une phase ordonnée dans l'alliage.

10. Procédé selon la revendication 9, dans lequel l'étape d'usinage thermomécanique consiste en un laminage à chaud, un laminage à mi-chaud, ou une combinaison de laminage à chaud et de laminage à mi-chaud.

11. Procédé selon la revendication 9, dans lequel l'étape d'usinage mécanique consiste en un laminage à chaud, un laminage à froid, ou une combinaison de laminage à chaud et de laminage à froid de la forme de produit allongée intermédiaire.
